



or alcohol, and this solution mixed with the emulsion. The following is an example of an emulsion made according to our invention:

A 0.001 molar solution of 2-thiouracil was made up in alcohol and this was added to a negative emulsion in the amount of from 0.001 to 1.0 gram of 2-thiouracil per 1000 cc. of emulsion. The pH of the emulsion was about 7.4. On incubation the fog produced in the emulsion was found to be much less than that produced in an emulsion under similar conditions not containing a fog inhibiting agent.

The amount of these fog inhibiting agents added to the emulsion is of importance since if too much of the fog inhibiting compound is added it may desensitize the emulsion markedly. The exact amount that must be used varies with the particular fog inhibiting compound selected and with the type of the emulsion used as regards grain size and alkalinity of the emulsion and ratio of the gelatin to silver halide. However, we have found that with gelatino silver halide, developing out emulsions, the amount of antifoggant will generally vary between about .001 gram and 1 gram of antifoggant per 1000 cc. of emulsion, although the amount may be as great as 5 grams of antifoggant per 1000 cc. of emulsion in some cases.

The fog inhibiting agents which we have found to be satisfactory may be used in various kinds of photographic emulsions. In addition to being useful in ordinary non-color-sensitized emulsions, they may also be used in ortho-chromatic and panchromatic emulsions or in X-ray emulsions. They can be used with or without sensitizing dyes and if used with sensitizing dyes may be added to the emulsion before or after them.

The following table will serve to illustrate the amounts of fog-inhibiting agents which we have found to be satisfactory, in each case the amount being used in 1000 cc. of a gelatino-silver halide emulsion containing from 5 to 10% gelatin:

|                                | Grams         |
|--------------------------------|---------------|
| 2-thiouracil                   | 0.001 to 1    |
| 2,6-dithiouracil               | .0003 to 0.3  |
| 7-methyl-2,6-dithiopurine      | .0005 to 0.05 |
| 7-methyl-6-thio-2-chloropurine | .0005 to .5   |
| 7-methyl-6-thiopurine          | .004 to .5    |
| 7-methyl-2,6,8-trithiopurine   | .001 to 0.1   |

It is to be understood that more or less of the fog-inhibiting agent than the amount stated above may be used. Generally, however, if a greater amount is used in the emulsion, either no increased fog-inhibiting effect is obtained, or there is a marked decrease in sensitivity of the emulsion.

In addition to fog-inhibiting action, some of

these compounds, such as 7-methyl-6-thiopurine and 7-methyl-6-thio-2-chloropurine, increase the sensitivity of the emulsion to some extent.

We consider as included within our invention all modifications and equivalents coming within the scope of the appended claims.

We claim:

1. A photographic emulsion comprising a colloidal material having a sensitive silver salt dispersed therein and containing a sulfur derivative of a pyrimidine selected from the group consisting of thiopurines and thiouracils in fog-inhibiting amounts.

15 2. A photographic emulsion comprising gelatin having a sensitive silver salt dispersed therein and containing a sulfur derivative of a pyrimidine selected from the group consisting of thiopurines and 2-thiouracils in fog-inhibiting amounts.

20 3. A silver halide gelatin emulsion containing a thiouracil in fog inhibiting amount.

4. A silver halide gelatin emulsion containing a mono-thiouracil in fog-inhibiting amount.

5. A silver halide gelatin emulsion containing 2-thiouracil in fog-inhibiting amount.

25 6. A photographic emulsion comprising a colloidal material having a sensitive silver salt dispersed therein and containing as an anti-foggant from about 0.001 gram to about 1 gram per liter of emulsion of a thiouracil.

30 7. A photographic emulsion comprising a colloidal material having a sensitive silver salt dispersed therein and containing as an anti-foggant from about 0.001 gram to about 1 gram per liter of emulsion of 2-thiouracil.

35 8. A gelatino silver halide emulsion containing as an anti-foggant from about 0.001 gram to about 1 gram per liter of emulsion of a thiouracil.

9. A gelatino silver halide emulsion containing as an anti-foggant from about 0.001 gram to about 1 gram per liter of emulsion of 2-thiouracil.

40 10. A silver halide gelatin emulsion containing a thiopurine in fog-inhibiting amount.

11. A silver halide gelatin emulsion containing a 6-thiopurine in fog-inhibiting amount.

45 12. A photographic emulsion comprising a colloidal material having a sensitive silver salt dispersed therein and containing as an anti-foggant from about .0005 gram to about 1 gram per liter of emulsion of a thiopurine.

50 13. A gelatino-silver halide emulsion containing as an anti-foggant from about .0005 to about 1 gram per liter of emulsion of a thiopurine.

14. A gelatino-silver halide emulsion containing as an anti-foggant from about 0.004 gram to about 0.5 gram per liter of emulsion of a 6-thiopurine.

SAMUEL E. SHEPPARD.  
WALDEMAR VANSELOW.